

May 1, 1945.

C. HARDY

2,374,747

METHOD OF MAKING TUBULAR BEARINGS

Filed March 9, 1942

3 Sheets-Sheet 1



INVENTOR  
Charles Hardy

BY  
Lannie Davis, Raymond L. Conner  
ATTORNEYS

May 1, 1945.

C. HARDY

2,374,747

METHOD OF MAKING TUBULAR BEARINGS

Filed March 9, 1942

3 Sheets-Sheet 2

Fig. 2.



INVENTOR  
Charles Hardy

BY  
Daniel, Davis, Rogow and Edmunds  
ATTORNEYS

May 1, 1945.

C. HARDY

2,374,747

METHOD OF MAKING TUBULAR BEARINGS

Filed March 9, 1942

3 Sheets-Sheet 3

Fig. 3,



INVENTOR  
Charles Hardy

BY  
Purcell, Davis, Neumann & Lamond

ATTORNEYS

## UNITED STATES PATENT OFFICE

2,374,747

## METHOD OF MAKING TUBULAR BEARINGS

Charles Hardy, Pelham Manor, N. Y., assignor to  
 Hardy Metallurgical Company, New York, N. Y.,  
 a corporation of Delaware

Application March 9, 1942, Serial No. 433,900

2 Claims. (Cl. 29—149.5)

This invention is concerned with the formation of metal linings in tubes and contemplates improvements in processes therefor. More particularly, the invention is concerned with the production from metal powder of annular linings in tubular bearings and the like.

Bearings comprising a tubular housing of relatively inexpensive and plentiful metal such as steel or iron and a thin annular lining of special bearing metal such as babbitt or bronze possess numerous advantages, not the least of which resides in the fact that they permit a great saving in strategic materials such as tin. However, it has not been practical heretofore to form thin annular linings in tubular bearings by powder metallurgy. I have developed a simple and practicable method whereby this may be accomplished and which assures that the metal powder will be adequately compacted against the tubular housing in which the lining is formed.

In accordance with my invention, a metal lining is formed on the inside of a tube by placing a layer of metal powder on the inside wall thereof and compacting the layer against the wall by squeezing a plastic core outwardly against the layer, the term "plastic" being employed to describe liquids and semi-solids such as water, oil, jelly, rubber, etc. Preferably the core is made of a resilient material such as rubber, and the squeezing action is brought about by compressing the core longitudinally of the tube, i. e., in the direction of the tube's axis.

The layer of metal powder may be placed on the inside of the tube in any convenient manner. Thus, the layer may be formed by pouring the metal powder into the annular space between the tube wall and a concentrically disposed core which has a cross-section less than that of the inside of the tube. The layer may also be formed by placing a loose mass of metal powder (with or without a binder) within the tube and spinning the tube on its axis so that the powder is forced against the tube wall by a centrifugal force sufficient in magnitude to cause the powder to adhere.

These and other features of my invention will be more thoroughly understood in the light of the following detailed description taken in conjunction with the accompanying drawings, in which:

Fig. 1 is a fragmentary vertical section taken through a press equipped with a rubber core and adapted to the practice of my invention;

Fig. 2 is a fragmentary vertical section taken through another type of equipment adapted to the practice of my invention and provided with

a hollow rubber core into which water or other fluid may be pumped; and

5 Fig. 3 is a fragmentary vertical section through still another type of apparatus for the practice of my invention and in which the core is entirely liquid.

Referring now to Fig. 1, it will be observed that the apparatus comprises a die 10 having a vertical bore into which a tubular bearing housing 11 to be lined is fitted snugly. A bottom punch 12 provided with an upwardly projecting guide pin 13 is disposed concentrically in the bore of the die. An annular rubber core 14 is disposed around the guide pin and extends within a short distance of the inside wall of the tubular bearing housing, so that there is left an annular space or powder fill 15 into which the metal powder that is to be compacted against the inside wall of the bearing housing is placed. A top punch 16, which corresponds in cross-section to the bottom punch and the rubber core, is disposed above the core and is adapted to push the rubber core downwardly against the bottom punch. A concentric bore in the top punch is adapted to receive the guide pin, so that the latter may slide therein.

In the operation of the apparatus of Fig. 1, the rubber core, mounted on the guide pin, is disposed in the position shown in the drawings, and the top punch is raised to a position higher than that shown in the drawings, so as to facilitate filling the annular space 15 with metal powder, for example a mixture of bronze powder with about 2% graphite. When the space has been filled, the top punch is brought down and compresses the rubber core downwardly and at the same time outwardly, since pressure tends to be transmitted in all directions in rubber and other semi-solids and liquids. The top and bottom punches then are forced together until a pressure of, say, 30 tons per square inch of punch cross-section is required for further movement, and this adequately and uniformly compacts the metal powder against the inside wall of the bearing housing to form a coherent and adherent annular layer. Thereafter, the top punch is raised and the rubber core shrinks to its original position (that shown in the drawings) leaving a substantial space between the lining and the core. At this point, a concentrically disposed ejection ring 17 which is journaled about the bottom punch is forced upwardly, so that the bearing housing with its adhering lining of compressed metal powder is pushed upwardly out of the die, from which latter position it may be removed.

After the lined bearing has been removed from

the die, it is subjected to a sintering operation to cause the particles of metal powder to become welded to each other and to the housing. In some instances, the sintered layer will be sufficiently uniform to serve as a bearing without any additional work. However, if desired, the bearing may be subjected to a coining operation. In such case, a punch that is somewhat larger in cross-section than that shown in Fig. 1 is forced longitudinally through the bearing to produce a smooth inside surface.

If desired, the sintered layer on the inside of the bearing may be machined on a lathe or other apparatus to bring it to requisite size and smoothness.

Referring now to Fig. 2, it will be observed that the apparatus comprises a die 20 with a vertical bore into which is fitted a tubular bearing housing 21. The apparatus is provided with an ejection punch 22 which is slideable in the bore of the die and has a recess 23 in its upper end. The apparatus is provided with an opposing or top punch 24 which is likewise slideable in the bore of the die and may be raised or lowered with respect thereto. The top punch is also provided with a concentric recess 25, the top of which is connected to a water pressure line or conduit 26 through which water may be pumped under pressure. Within the recess of the top punch and extending below it is a hollow rubber sack or core 27. This core is fastened firmly into the upper recess around the water pressure line and is closed at the other end so that it forms a cylindrical sack. The cross-section of the sack in the undistended condition is slightly less than the inside bore of the tubular bearing housing.

In the operation of the apparatus of Fig. 2, a layer 28 of metal powder is disposed in the tubular bearing housing before the bearing housing is placed in the apparatus. This may be done conveniently by placing loose metal powder in appropriate amount and accompanied by a suitable binder, for example lacquer, in the housing and then spinning the housing on its axis to cause the powder to spread over the inside surface and fill the annular groove 29. With the bearing thus lined with a coherent but substantially uncompacted layer of metal powder, it is disposed in the apparatus on the ejection punch, and the top punch is lowered so that the rubber core extends through the bore of the bearing housing. With the ejection punch and the top punch held in these positions, water or other fluid is pumped in through the water pressure line so that the rubber core is distended and squeezes the metal powder layer against the wall of the housing. The pressure within the apparatus is built up to, say, 20 tons per square inch of inside bearing surface. The water pressure is then reduced, as by pumping the water out of the apparatus. This causes the core to shrink away from the compacted lining of the housing. The top punch and the core are then withdrawn from the apparatus and the line bearing is ejected from the die by forcing the ejection punch upwardly.

The line bearing produced in the apparatus of Fig. 2 is subjected to a sintering operation as described in the case of Fig. 1. Thereafter, the sintered bearing may be subjected to a coining or machining operation to improve its bearing surface, i. e., the inside of the lining.

It will be observed that in the apparatus of Fig. 2 the pressure is exerted in all directions and particularly outwardly toward the wall of the bearing housing, so that the powder layer is uni-

formly and thoroughly compacted against the inside wall of the housing.

To consider the apparatus of Fig. 3, a tubular bearing housing 30 is disposed with a relatively snug fit in the vertical bore of a die 31 after the bearing housing has had applied to it a powder layer 32. The annular powder layer may be formed in the bearing housing in any convenient method, for example by the centrifugal operation described in the case of the apparatus of Fig. 2. In the die, the bearing housing rests on a bottom punch 33 which fits snugly in the bore of the die, but is slideable therein. After the housing is so positioned, a top punch 34 is slid into the top of the die, where it fits snugly on the top of the bearing housing. Then liquid, for example oil or water, is pumped into the top punch through a concentric supply conduit 35. This forms a liquid core 36 inside the powder layer and forces the powder layer outwardly against the wall of the bearing housing with any desired pressure, said 30 tons per square inch.

In order to bring about a more adequate compacting of the powder in the housing, a tubular insert 37 of cardboard, thin metal, or other relatively flexible material may be placed inside the lined bearing housing before the compression step.

After the compression has been accomplished 30 by pumping the liquid into the core, the pressure is released and the upper top punch and the bottom punch are both raised and the bearing with its compacted lining is removed from the apparatus and subjected to sintering and the other 35 subsequent treatments already described.

My invention is applicable to the lining of very long tubes, although in most applications, for example bearings, the tubes will be relatively short. However, irrespective of the length of the 40 tube, it is possible to obtain an equalization of lateral pressure so that the powder layer inside the tube is uniformly compacted in all areas.

The tube to be lined may be of any appropriate metal and may be thick or thin. In all 45 cases the die should be sufficiently strong to "back-up" the tube adequately.

For long tubes, the apparatus of Fig. 2 and Fig. 3 are preferable. The apparatus of Fig. 1 is particularly useful in the compression of powder layers within relatively short tubes, when it is not necessary to obtain absolute equality of pressure over a long length of tube.

I claim:

1. In the formation of a metal lining on the 55 inside wall of a tube, the improvement which comprises placing a mass of discrete metal powder particles on the inside wall of the tube, forming the mass of metal powder particles into a layer, placing a plastic core in the tube inside 60 the space occupied by the powder, and compacting the layer of powder against the interior wall of the tube by squeezing the plastic core outwardly against the wall.

2. In the formation of a metal lining on the 65 inside wall of a tube, the improvement which comprises forming an annular layer of discrete metal powder particles on the inside wall of the tube by spinning the tube on its axis so that the powder is forced against the wall thereof, placing a plastic core in the tube inside the space 70 occupied by the powder, and compacting the layer of powder against the interior wall of the tube by squeezing the plastic core outwardly against the wall.

CHARLES HARDY.